

O. R. WITTER.  
SHOE STIFFENER BLANK.  
APPLICATION FILED NOV. 12, 1917.

1,283,391.

Patented Oct. 29, 1918.

Fig. 1.



Fig. 2.



Fig. 3.



Fig. 4.



Fig. 5.



INVENTOR:  
O. R. Witter  
by Wright Brown & Company  
ATTYS.

# UNITED STATES PATENT OFFICE.

OSBORNE R. WITTER, OF SWAMPSOFT, MASSACHUSETTS, ASSIGNOR OF ONE-HALF TO  
AUGUST H. GOETTING, OF SPRINGFIELD, MASSACHUSETTS.

## SHOE-STIFFENER BLANK.

1,283,391.

Specification of Letters Patent. Patented Oct. 29, 1918.

Application filed November 12, 1917. Serial No. 201,416.

*To all whom it may concern:*

Be it known that I, OSBORNE R. WITTER, a citizen of the United States, residing at Swampscott, in the county of Essex and 5 State of Massachusetts, have invented new and useful Improvements in Shoe-Stiffener Blanks, of which the following is a specification.

This invention relates to blanks for box-toes and heel counters for shoes, and has for 10 its object to provide a blank which is waterproof, and is adapted to be pulled over and conform to portions of a last without liability of tearing the pulled over portion, the 15 cost of the blank being materially less than that of any blank heretofore known, so far as I am aware, having the above-mentioned characteristics.

The invention consists in the improvements which I will now proceed to describe 20 and claim.

Of the accompanying drawings, forming a part of this specification,—

Figure 1 is a side view of a box-toe blank 25 embodying the invention.

Fig. 2 is a section on line 2—2 of Fig. 1.

Fig. 3 is a side view of a heel counter blank.

Fig. 4 is an enlargement of a portion of 30 Fig. 2.

Fig. 5 is a section on line 5—5 of Fig. 3, showing by dotted lines one edge portion of the blank turned or molded to form a counter flange.

35 The same reference characters indicate the same or similar parts in all of the figures.

My improved stiffener includes an inner layer 12 made from a vulcanizable compound containing rubber, sulfur and suit-

40 able ingredients giving body to the layer.

The said ingredients may comprise ground frictioned fabric such as duck or canvas (waste pieces being employed), lime, and litharge, the several ingredients being pro-

45 portioned to produce a compound which will be rendered semi-hard by vulcanization.

I use a greater proportion of sulfur than would be used in a compound which is relatively elastic when vulcanized, my aim being 50 to produce a relatively cheap compound which is waterproof and has sufficient stiffness to resist crushing pressure.

To one side of the layer 12 I apply an outer layer 13 of textile fabric, such as rela-

55 tively thin duck or canvas, the preferred

grade being what is known as eight-ounce duck, although I may use either lighter or heavier fabric. The layer 12 is applied to the layer 13 before the composition of the layer 12 is vulcanized, the outer layer 13 being 60 preferably frictioned and thus not only rendered waterproof, but also adapted for firm union to the inner layer by the simultaneous vulcanization of the frictioned material and of the material of the inner layer. 65

The assembled layers are then subjected to vulcanizing heat and pressure and are thus caused to adhere firmly to each other, the inner layer at the same time being rendered semi-hard and adapted for reduction 70 by a skiving knife.

I next skive the inner layer 12 from its relatively thick central portion to the margin of the outer layer 13, and thus provide the blank with a flexible edge formed mainly 75 by the margin of the outer layer, which margin has a sufficient degree of tensile strength and is waterproof because of the frictioning material.

The portion of the blank formed by the 80 marginal portion of the outer layer and the skived portion of the inner layer, is flexible and extensible, its flexibility and extensibility decreasing from the margin of the blank inwardly, so that the central portion of the 85 blank is relatively thick and stiff and is adapted to resist indenting or crushing pressure when the blank has been conformed to a last, while the margin is adapted to be stretched and pulled over into conformity 90 to the surface of the last. The tensile strength of the outer layer enables the marginal portion of the blank to withstand pulling over strains.

The improved blank above described is 95 adapted to be converted by the usual methods into a stiffener conforming to various parts of a last, unaffected by moisture, and adapted to resist pressure tending to indent its outer surface.

While I do not limit myself to any particular compound for the layer 12, the compound may be composed of the following ingredients in substantially the following proportions by weight:

Ground fabric, twenty-five parts,

Ground cured scrap rubber, twenty-five parts,

Reclaimed rubber, fourteen parts,

Litharge, one and one-half parts,

100

105

110

Lime, one part,  
Red oxid of iron, or other coloring matter, ten parts,

- 5 Asbestos fiber, seven parts,  
Sulfur, one and one-half parts.

When the invention is applied to a heel counter I have found it advisable to mold the blank into a formed counter before insertion of the same into a shoe, and therefore to provide means which will hold the same in its molded form and resist the tendency due to the resilience of the material to revert to the form of the blank. The means for accomplishing this further result 10 consists in a composition which is applied in a plastic state to the skived edge of the blank which later forms the flange of the molded counter; such composition when dried or cooled being firm and having a 15 binding effect upon the molded flange.

Suitable compositions for this purpose are compounds containing glue or paraffin wax, or other materials of the sort which become fluid when heated or dissolved, or becomes 20 solid upon cooling or drying. The lower skived edge of the blank made in the manner previously described, is coated at 14 with such a composition, and thereafter the blank is formed in a counter-molding machine, the 25 dies of which are preferably heated in order to soften the composition while the molding action takes place, permitting the coated edge of the blank to be turned inward or outward, as the case may be, to make the 30 flange of the counter, without cracking. The composition thereafter hardening, retains 35 the counter in its molded condition.

I claim:

1. A shoe stiffener blank including an 40 inner waterproof layer composed of a compound containing rubber and sulfur rendered semi-hard by vulcanization, and at the same time prepared for marginal reduction by a skiving knife, and an outer layer of 45 flexible and extensible textile fabric united to the inner layer by the vulcanization of the latter, the inner layer being marginally skived to render the marginal portion of the blank relatively flexible, extensible and 50 formable, while the central or body portion is relatively stiff and adapted to resist crushing pressure.

2. A shoe stiffener blank including an in-

ner waterproof layer composed of a compound containing rubber and sulfur, rendered semi-hard by vulcanization, and at the same time adapted for reduction by a skiving knife, and an outer waterproof layer of flexible and extensible frictioned textile fabric caused to adhere to the inner layer by the vulcanization of the latter, and of the frictioning material, the inner layer being marginally skived from its relatively thick central portion to the margin of the outer layer to provide the blank with a flexible waterproof edge formed mainly by the margin of the frictioned outer layer, the portion of the blank formed by the marginal portion of the outer layer and the skived portion of the inner layer being flexible and extensible, and its flexibility and extensibility decreasing from the margin of the blank inwardly, so that the central portion of the blank is relatively thick and stiff and adapted to resist crushing pressure, while the margin is adapted to be stretched and pulled over into conformity to surfaces of a last, the tensile strength of the outer layer enabling said portion to withstand pulling over strains.

3. A shoe stiffener blank including an inner waterproof layer composed of a compound containing rubber and sulfur rendered semi-hard by vulcanization, and an outer layer of flexible and extensible textile fabric united to the inner layer by the vulcanization of the latter, the inner layer being marginally skived and having upon one of its skived portions a coating of material which is normally solid and is adapted to be rendered fluid or plastic.

4. A shoe stiffener formed from a blank including an inner waterproof layer composed of a compound containing rubber and sulfur rendered semi-hard by vulcanization, and an outer layer of flexible and extensible textile fabric united to the inner layer by the vulcanization of the latter, the inner layer being marginally skived and the blank being molded into the desired shape, one of the skived marginal portions forming a flange, and said flange being coated and retained in form by a binding composition.

In testimony whereof I have affixed my signature.

OSBORNE R. WITTER.